

Patented June 10, 1924.

1,497,265

# UNITED STATES PATENT OFFICE.

JOSEPH HAAS, JR., OF MUNCIE, INDIANA, ASSIGNOR TO THE ROESSLER AND HASS-LACHER CHEMICAL COMPANY, OF NEW YORK, N. Y., A CORPORATION OF NEW YORK.

## ZINC-ELECTROPLATED ARTICLES.

No Drawing. Original application filed September 16, 1922, Serial No. 588,567. Divided and this application filed January 19, 1923. Serial No. 613,760.

To all whom it may concern:

Be it known that I, JOSEPH HAAS, Jr., citizen of the United States, and resident of Muncie, in the county of Delaware and State of Indiana, have invented certain new and useful Improvements in Zinc-Electroplated Articles, of which the following is a specification.

My invention relates in general to the electroplating of zinc or its alloys upon iron or steel in cyanid baths. Such cyanid plating baths are widely used because of their greater throwing power as compared with other baths which have been proposed for zinc plating.

Hitherto the commercial zinc plating of ferrous articles in cyanid baths has been subject to certain limitations. For example, it has been considered impracticable in cyanid baths to zinc plate iron castings at all. Moreover, the plating of articles of wrought iron or wrought steel has been attended with some difficulty in respect to articles of irregular surface, the difficulty being that those portions of the article which are more remote from the anode receive too thin a coating. In the plating of small ferrous articles this difficulty becomes so pronounced that hitherto it has been deemed impracticable to zinc plate such articles by the basket method in cyanid baths.

In investigations to determine the cause of these difficulties, I have found that it is due to the relatively low discharge potential of hydrogen upon cast iron, which causes hydrogen to be deposited rather than zinc. It has also been observed in plating cast iron and steel in the same bath, that more hydrogen is evolved upon the cast iron than on the steel, evidencing that the discharge potential of hydrogen on cast iron is much lower than that of hydrogen on steel. This is further evidenced by the common practice in plating copper on cast iron to use less free cyanid than in plating on steel, too much cyanid in either case causing only evolution of hydrogen.

In order to successfully deposit zinc on cast iron in a cyanid bath, the factors to be considered are the discharge potential of hydrogen; the electrode potential of the cathode metal; and the electrode potential of the metal to be deposited, all three being affected by the crystalline structure of the cast iron.

cathode. The general rule may be said to be that if the discharge potential of hydrogen on the cathode metal is low, or below the electrode potential of the deposited metal, and the difference between the electrode potential of the deposited metal and the discharge potential of hydrogen is great, hydrogen only is deposited. If the difference is not great, both hydrogen and metal are deposited while if the discharge potential of hydrogen considerably exceeds the electrode potential of the deposited metal, the metal alone is deposited.

Where cast iron is first plated with copper or nickel, zinc can readily be deposited from a cyanid bath, due to the discharge potential of hydrogen being raised, but this is an added expense, and coatings of copper or nickel on cast iron are likely to be porous, and when porous are not corrosion-preventative but stimulate corrosion.

The problem is solved according to this invention by bringing the discharge potential of hydrogen closer to the potential of zinc in a cyanid bath without an extra electroplating bath, by depositing the zinc in the presence of a metal electrochemically active to prevent corrosion. Such a metal is mercury which has the effect in a cyanid electroplating bath of bringing the discharge potential of hydrogen so near the potential of zinc that zinc will be deposited together with a small percentage of mercury. In other words, the presence of mercury has the effect of making the difference between the discharge potential of hydrogen and the potential of zinc so much less than the difference between the discharge potential of hydrogen on cast iron and the potential of zinc, as to secure a good deposit of zinc on cast articles not heretofore satisfactorily coated with zinc by electroplating.

Other improvements result from my invention among which are the following:

1. The color, smoothness, fineness of grain structure, resistance to corrosion, and hardness of the zinc mercury deposit are superior to those formerly obtained of zinc alone from cyanid baths.
2. The current efficiency at the cathode is markedly increased.
3. The anode wastage due to chemical corrosion is decreased.
4. The zinc coatings do not readily stain.

in the solution or when dried out, or when subsequently handled during assembling.

As illustrations of my invention, I will now describe the same as applied to the zinc plating of various types of iron and steel articles.

*Example I.*—To plate gray or white iron castings such as pipe fitting, for example, I proceed as follows:

10 The fitting is first cleaned, preferably by sand blasting, until all of the scale and loose dirt are removed, and a clean iron surface is exposed. Should the surface of the fitting again become rusted, or otherwise fouled 15 and dirty before going to the plating tank, it should then be again cleaned preferably by dipping in muriatic acid solution of about 1.09 specific gravity after which it is rinsed in a hot caustic solution containing 20 one to five per cent NaOH until ready for the plating operation.

The fitting so cleaned may then be dipped in a mercury solution containing for example:

25 Mercuric chloride ..... 4 oz.  
Nitric acid, sp. g. ..... 1.4  $\frac{1}{2}$  oz.  
Water to make ..... 1 gal.

The fitting is then immediately suspended 30 in a zinc cyanid plating solution to which has been added a small amount of a soluble mercury compound. Excellent results are obtained from a bath of the following composition:

35 Water ..... 1 gal.  
Zinc cyanid ..... 4 oz.  
Sodium cyanid ..... 4 oz.  
Sodium hydroxid ..... 2 oz.  
Mercuric oxid .....  $\frac{1}{2}$  oz.

40 The solution is maintained at a temperature of from 40° to 50° C. Although in this species of the process, the mercury is first coated on the cathode, the coating is 45 of zinc and mercury even if the mercury salt is omitted from the bath as one permeates the other. In a thick deposit, the zinc at the outside may be practically free 50 of mercury, but such thick coating is not ordinarily desired. The preferred voltage is from three to six volts depending upon the quantity of work being plated. When the required deposit has been secured, the fitting is removed from the solution, rinsed 55 in cold and hot water successively, and then air dried. The bath must be replenished from time to time as the several ingredients become depleted, but the amount of mercury where used in the bath must not be permitted to become excessive inasmuch as the 60 permanence of the coating will be impaired.

*Example II.*—To plate large articles of wrought iron or wrought steel, such as automobile rims, the article instead of being sand blasted, is cleaned by pickling alter-

nately in alkaline and acid cleaning solutions until a chemically clean metallic surface is exposed. It may then be dipped in the mercury solution and plated as described in Example I. When plated, the rim is 70 rinsed in cold and hot water, and air dried. The deposits thus obtained are tough and of pleasing appearance and are more resistant to corrosion and abrasion than any hitherto obtained in the art.

75 *Example III.*—To plate burrs, bolts, screws, and other small articles of iron or steel, I proceed as in Example II, except that the articles are handled throughout in coarse-meshed wire baskets and are plated 80 with a current of full six volts. The deposits obtained are of excellent color and durability; moreover, the plate is of uniform thickness throughout all parts of the basket.

85 As I believe I am the first to discover a means for increasing the potential of the cathode in zinc cyanid plating, and thereby reducing evolution of hydrogen and increasing the amount and quality of the coating, 90 besides producing a novel coating, I do not limit myself to any specific way of introducing the mercury except as specifically required by the appended claims.

95 Within the broad scope of the invention, I have obtained similar results by dipping the cathode first in a solution of a mercury salt and then plating in an ordinary cyanid bath without added mercury salt; and by plating in a cyanid bath with added mercury salt without preliminary dipping. In the former case, the mercury becomes alloyed with the first zinc deposited but upon continued plating, the percentage of mercury diminishes, and finally the coating may 100 be practically pure zinc. With mercury in the bath, the coating is uniformly alloyed with from 1.5% to 2.0% of mercury. The most resistant and satisfactory coatings have about 2.0% of mercury. If the percentage 105 is below about 0.2%, the advantages resulting from its use are small, and the use is limited. If the percentage of mercury is above about 5.0%, the coatings are unsatisfactory in texture, are brittle, and of little 110 utility. I do not limit myself to the aforesaid mercury compounds as I may use any soluble mercury salt for the dip which will deposit metallic mercury on the cathode, and any mercuric compound which is soluble in 115 the bath. The oxide is preferred for the bath because it introduces into the bath no foreign anion. Mercurious compounds are not recommended for the bath as they are in part reduced by the bath with the precipitation of metallic mercury. In the pre-

120 liminary dip solution and in the bath I may use other soluble mercury salts such as nitrate, sulphate, etc.

125 This application is a division of my ap-

plication Ser. No. 588,567, filed September 16, 1922, wherein is broadly claimed the novel process of depositing mercury in the presence of zinc on a ferrous cathode, the claims herein being restricted to the novel product resulting from the process therein described.

I claim:

1. As a new article of manufacture, a ferrous article coated with a dense bright

electrolytic coating comprising zinc alloyed with mercury.

2. As a new article of manufacture, a ferrous article coated with a dense bright electrolytic coating comprising zinc alloyed <sup>15</sup> with between 0.2% and 5.0% of mercury.

Signed at Perth Amboy, in the county of Middlesex and State of New Jersey, this 13th day of January, A. D. 1923.

JOSEPH HAAS, JR.